

G. PALMER.  
PRINTER'S BLANKET.  
APPLICATION FILED JAN. 16, 1913.

1,147,969.

Patented July 27, 1915.

*Fig. 1.*



*Fig. 2.*



*Fig. 3.*



Attest:

J. D. Mitchell  
L. C. Morrison

George Palmer Inventor:  
by  
Jos. H. Freeman, Atty

# UNITED STATES PATENT OFFICE.

GEORGE PALMER, OF CHICAGO, ILLINOIS, ASSIGNOR TO GEORGE L. WILLSON, OF NEW YORK, N. Y.

## PRINTER'S BLANKET.

1,147,969.

Specification of Letters Patent. Patented July 27, 1915.

Application filed January 16, 1913. Serial No. 742,372.

To all whom it may concern:

Be it known that I, GEORGE PALMER, a citizen of the United States, and a resident of Chicago, Cook county, State of Illinois, have invented certain new and useful Improvements in Printers' Blankets, of which the following is a specification.

The invention relates to printers' blankets, and has for an object to provide an improved construction of the character referred to which shall be highly efficient and economical in operation.

Other objects of the invention will be apparent from the following description.

The invention consists in the novel improvements, features of construction, and combinations of elements hereinafter more fully set forth.

In the accompanying drawings, which are referred to herein and form part hereof, are illustrated several embodiments of the invention, the same serving in connection with the description more fully to explain the invention.

Of the drawings: Figure 1 is a cross-section of a portion of a printer's blanket constructed in accordance with the invention; Fig. 2 is a similar view of a modification; and Fig. 3 is a similar view of another modification.

Referring now in detail to the drawings, the embodiment of the invention illustrated in Fig. 1 comprises a body 5 of yielding material. While, as far as certain other features of the invention are concerned, said body may be made of various materials, it is a feature of the invention to employ felt for said body because of its peculiar fitness, said felt preferably being the same as that ordinarily used in rotary presses for newspaper work. Suitable means are provided to prevent the felt from stretching while on the press and from becoming matted or otherwise deteriorating from use. While this may be done in various ways and by using divers agents, preferably and as shown and in accordance with another feature of the invention, the felt is impregnated with a composition which has more or less elasticity and yet is impervious to oil. The preferred composition comprises glue, glycerin, plaster of Paris, and chicle gum in suitable proportions as, say: eight parts of glue; two parts of glycerin; two parts of plaster of Paris; and two parts of chicle.

The glycerin keeps the glue from hardening and forms therewith an elastic compound similar to rubber but differing therefrom in that it is not injuriously affected by the oil or varnish or other ingredients commonly used in printer's ink. The plaster of Paris and chicle add body to the composition and prevent undue softening by heat. The impregnation of the felt need not be complete but may obtain to any suitable extent, preferably and as illustrated in the drawings extending practically through about three-fourths of the felt, see that portion of the blanket indicated by the numeral 6.

Preferably and as shown, see Fig. 2, a piece of canvas 7 is attached to the back of the felt to give the same greater power of resistance to wear and particularly to resist stretching; and, if desired, a thin rubber blanket comprising one or more layers of rubber 8 or canvas 9, such as the rubber blankets employed on the said presses, may be secured to the back of the felt, and this canvas 7 or blanket 8, 9 may be secured either by the composition with which the felt is impregnated or by a rubber cement or other suitable adhesive. When the rubber is used back of the impregnated felt in this manner, it is protected from the injurious effects of the oils and other ingredients of the ink by the glutinous composition.

It will be seen that a printer's blanket constructed in accordance with the invention will carry out the objects of the invention besides possessing other advantages which will be apparent to those skilled in the art.

The invention in its broader aspects is not limited to the precise constructions or proportions of parts shown and described nor to any particular constructions by which the same has been or may be carried into effect, as many changes may be made in the details thereof without departing from the main principles of the invention or sacrificing its chief advantages.

I claim:

1. A printer's blanket including a nap-carrying element, a woven fabric, and an interposed compound comprising an oil-resisting mass consisting of glycerized glue combined with a heat-resisting mass consisting of plaster of Paris and chicle.

2. A printer's blanket including a nap-carrying element, a woven fabric, and an interposed compound comprising an oil-

100

105

110

resisting mass consisting of glycerized glue combined with a heat-resisting mass consisting of plaster of Paris and chicle in minor proportion relatively to the oil-resisting mass.

3. A printer's blanket including a nap-carrying element, a woven fabric, and an interposed compound comprising an oil-resisting mass consisting of glue and glycerin 10 in major proportion combined with a heat-resisting mass consisting of plaster of Paris and chicle.

4. A printer's blanket including a glutinous compound comprising an oil-resisting mass of glycerized glue combined with a heat-resisting mass of plaster of Paris and chicle, and an adherent nap-carrying fabric impregnated with said compound on one 15 side and to an extent approximately more than one half of its thickness.

5. A printer's blanket including a layer of felt partially impregnated with a glutinous compound comprising an oil-resisting mass of glycerized glue and a heat-resisting mass of plaster of Paris and chicle 20 in minor proportion relatively to the oil-resisting mass.

6. A printer's blanket including a layer of felt coated on one side only with a glutinous compound including an oil-resisting mass of 25 glycerin and glue combined with a heat-resisting mass of plaster of Paris and chicle in minor proportion relatively to the oil-resisting mass.

30 7. A printer's blanket composed of a layer of felt coated on one side only with a glutinous compound including an oil-resisting mass of glycerin and glue combined with a heat-resisting mass of plaster of Paris and 35 chicle in minor proportion relatively to the

oil-resisting mass, and a layer of canvas adhering to the compound.

8. A printer's blanket comprising a strip of felt impregnated with a compound composed of eight parts glue, two parts glycerin, 45 two parts plaster of Paris, and two parts of chicle.

9. A printer's blanket comprising a strip of felt partly impregnated with a compound composed of eight parts glue, two parts 50 glycerin, two parts plaster of Paris, and two parts chicle.

10. A printer's blanket composed of a layer of felt of relatively great thickness, a glutinous compound with which one side of 55 the felt is coated and penetrating said felt to more than half of its thickness, said compound including an oil-resisting mass of glycerized glue combined with a heat-resisting mass of plaster of Paris and chicle in 60 minor proportion relatively to the oil-resisting mass, a layer of canvas adhering to the compound, a layer of rubber adhering to the canvas, and a second layer of canvas attached to the layer of rubber.

65 11. A printer's blanket including a layer of felt coated on one side with a glutinous compound including an oil-resisting mass of glycerin and glue combined with a heat-resisting mass of plaster of Paris and chicle, 70 a layer of canvas adhering to the compound, and a layer of woven fabric cemented to the canvas.

In testimony whereof, I have signed my name to this specification, in the presence of 75 two subscribing witnesses.

GEORGE PALMER.

Witnesses:

Miss R. SNIDERMAN,  
ADDISON D. KELLEY.